

## [54] PROCESS FOR DESULFURIZING COKE

[75] Inventor: Mahendra T. Thakker, Ponca City, Okla.

[73] Assignee: Continental Oil Company, Ponca City, Okla.

[22] Filed: Apr. 16, 1971

[21] Appl. No.: 134,909

## Related U.S. Application Data

[63] Continuation-in-part of Ser. No. 799,150, Feb. 10, 1969, abandoned.

[52] U.S. Cl. 208/46, 208/131, 201/17

[51] Int. Cl. C10g 9/14, C10b 57/00

[58] Field of Search 208/46, 106, 127, 131; 201/17

## [56] References Cited

## UNITED STATES PATENTS

|           |         |                    |          |
|-----------|---------|--------------------|----------|
| 2,921,017 | 1/1960  | Johnson et al..... | 208/106  |
| 2,721,169 | 10/1955 | Mason et al.....   | 23/209.9 |
| 2,872,384 | 2/1959  | Nelson et al.....  | 201/17   |
| 3,009,781 | 11/1961 | Johnson et al..... | 201/17   |
| 3,179,584 | 4/1965  | Hamner et al.....  | 208/106  |

Primary Examiner—Herbert Levine  
Attorney—Joseph C. Kotarski et al.

## [57] ABSTRACT

Petroleum coke of reduced sulfur content is produced by adding an alkali metal carbonate (preferably sodium carbonate) to the coker feedstock prior to coking and then, after coking, treating the coke with hydrogen at an elevated temperature.

7 Claims, 1 Drawing Figure



PATENTED MAR 27 1973

3,723,291



INVENTOR.  
MAHENDRA T. THAKKER

BY

*Jerry B. Keeler*

ATTORNEY

## PROCESS FOR DESULFURIZING COKE

## CROSS-REFERENCE TO RELATED APPLICATIONS

This application relates to my application Ser. No. 799,151 entitled "PROCESS FOR DESULFURIZING COKE" filed Feb. 10, 1969 and is a continuation-in-part of Ser. No. 799,150 filed Feb. 10, 1969 and both now abandoned.

## BACKGROUND

This invention is a process for producing coke of reduced sulfur content by adding an alkali metal carbonate (or mixtures of such carbonates) to the coker feedstock and then, after coking, treating the coke with hydrogen at an elevated temperature.

The importance of coke desulfurization processes will undoubtedly increase as air pollution regulations result in the establishment of coke specifications including lower sulfur contents. The problem is accentuated by the present trend toward the use of higher sulfur content crude oils in many oil refineries.

One method of reducing the sulfur content of a coke is to reduce the sulfur content of the feed to the coker, either by careful selection of feedstocks or by desulfurization of the feedstock. Another method involves the desulfurization of the coke itself. This invention concerns the latter alternative.

## DESCRIPTION OF THE PRIOR ART

The prior art suggests methods of desulfurizing petroleum coke by the addition of sodium carbonate to the coke, followed by heat treatment. For example, see the following references: *Ind. Eng. Chem.*, Vol. 52, No. 8, pp 675-677 (1960); U.S. Pat. No. 3,387,941.

U.S. Pat. No. 3,179,584 shows addition of sodium carbonate to coker feedstock to increase the production of hydrogen in the coking process, but desulfurization is not disclosed or suggested.

U.S. Pat. No. 2,921,017 suggests mixing sodium carbonate with a coker feedstock in order to produce a coke of reduced sulfur content; however, the patentee does not disclose the use of hydrogen.

The prior art also suggests desulfurization of coke by hydrogenation, as for example: U.S. Pat. No. 3,130,133; *Ind. Eng. Chem.*, Vol. 52, No. 7, pp 599-600 (1960); U.S. Pat. No. 2,768,939.

The prior art also shows the desulfurization of coke by treatment with hydrogen in the presence of materials other than sodium carbonate, e.g.: U.S. Pat. Nos. 2,824,047 and 3,101,303.

The prior art also teaches that petroleum fractions generally can be used for coking feedstocks. The prior art also has recognized that certain reduced crudes, thermal tars including tars from ethylene and other olefin processes are superior as feedstocks when a needle like or premium coke is desired. While the art recognizes that any hydrocarbon can be used as a coking feedstock, the lower molecular weight materials generally are more valuable for other purposes and the heavy resids and tars, having a high carbon content are more suitable and are more easily coked. The choice of feedstocks then depends upon economies and type of coke desired, the choice being within the skill of the art.

## BRIEF SUMMARY OF THE INVENTION

This invention is a process for producing coke of reduced sulfur content by adding an alkali metal carbonate (or a mixture of such carbonates) to the coker feedstock and then, after coking, treating the coke with hydrogen at an elevated temperature. Sodium carbonate is preferred because it is cheap, although other alkali metal carbonates could be used.

10 Sodium carbonate is mixed directly with the coker feedstock and the feedstock is then coked. After the coking operation is completed, the coke is ground to a particle size sufficiently small that the hydrogenation treatment will be effective, and preferably sufficiently small so that the coke can be fluidized during hydrogenation.

15 After the hydrogenation step, the coke is washed with water in order to remove the carbonate.

## DESCRIPTION OF THE DRAWING

The drawing shows a simplified flow diagram illustrating the process.

## DETAILED DESCRIPTION OF THE DRAWING

Referring to the drawing, a suitable conventional coking feedstock is passed to mixer 1, in which sodium carbonate is blended into the feedstock. The resulting mixture is passed to coker 2 (for example, a conventional delayed coker) which is operated under conventional coking conditions. The green coke is ground in crusher 3 to a particle size of less than 12 U.S. Standard mesh, preferably -50 to +100 Standard U.S. mesh. The particles of greater than 12 mesh are separated into separator 4 and recycled to the crusher. The ground coke is then conveyed to desulfurizer 5, into which hydrogen is introduced through line 6. The desulfurizer is preferably operated so as to maintain the coke bed in a fluidized condition. The overhead vapors are passed through a conventional  $H_2S$  scrubber 7 from which recycle hydrogen is recovered through line 8. The desulfurized coke, after washing with hot water in washer 10, may then be passed to a calciner (not shown). The preferred conditions are as follows:

Amount of sodium carbonate (added to coker feedstock): 0.3 to 5 percent, preferably 0.3 to 1 percent, based upon coke obtained (line 9 of drawing), depending upon the amount of sulfur in the coke.

Hydrogenation treatment temperature, °F: at least about 1,000°F, to about 2,000°F, preferably about 1,000° to 1,600°F and most preferably about 1,100°F to 1,400°F.

Hydrogenation pressure, atm: any convenient pressure is satisfactory. Atmospheric pressure is satisfactory although higher pressures are preferable.

Hydrogenation treatment time, hours: at least 2 hours, preferably 3 to 8 hours, and most preferably 4 hours, for low sulfur cokes. For high-sulfur cokes, treating times of up to 16 hours may be required, preferably 8-12 hours.

The particular set of conditions selected will, of course, depend upon the sulfur content of the coker feedstock and the desired degree of sulfur removal. The preferred set of conditions for the hydrogen treat-

ment of low-sulfur feedstocks is a 4-hour treatment at about 1,200°F. For high sulfur coke (greater than 2 percent), the treatment time should be increased to obtain the desired reduction in sulfur content.

The process may be carried out as a batch or continuous operation.

In the following tables, the particle sizes refer to U.S. Standard mesh. The coker feedstock was reduced crude. Table I illustrates the effectiveness of this process. In Run No. 1, sodium carbonate was added to the coke, whereas in all other runs, it was added to the coker feedstock.

In all the tables, the final ash content was measured after washing the coke with water.

A comparison of runs from the above table with that of Table II shows at a given temperature, the improvement in coke removal is substantial. At 1,600°F, runs 12 and 20, the improvement was 29.9 percent. How-

ever, as we increase temperature, the total sulfur removed becomes less and therefore about 2,000°F is a practical upper limit.

It is also pointed out, as is known in the prior art, that the nature of the coking feedstock, or rather the resulting coke, will determine the optimum hydrogenation temperature for desulfurization. With the particular feedstock, e.g., the particular reduced crude, showed an optimum temperature at about 1,200°F both with the prior art method and the invention method. With

15

TABLE I.—COKE MADE BY ADDITION OF  $\text{Na}_2\text{CO}_3$  TO REDUCED CRUDE

| Run number                             | 1            | 2            | 3            | 4            | 5            | 6            | 7            | 8            | 9            |
|----------------------------------------|--------------|--------------|--------------|--------------|--------------|--------------|--------------|--------------|--------------|
| Particle size                          | -50+100      | -30+100      | -30+100      | -30+100      | -30+100      | -30+100      | -30+100      | -30+100      | -30+100      |
| Percent $\text{Na}_2\text{CO}_3$ added | *4           | 0            | 5            | 4.57         | 2.17         | 1.32         | 0.634        | 0.335        | 0.7          |
| Fluidizing gas                         | $\text{H}_2$ | $\text{H}_2$ | $\text{H}_2$ | $\text{H}_2$ | $\text{H}_2$ | $\text{H}_2$ | $\text{H}_2$ | $\text{H}_2$ | $\text{H}_2$ |
| Temperature, °F                        | 1,200        | 1,200        | 1,200        | 1,200        | 1,200        | 1,200        | 1,200        | 1,200        | 1,000        |
| Pressure, atm                          | 1            | 1            | 1            | 1            | 1            | 1            | 1            | 1            | 1            |
| Velocity of gas, ft./sec.              | 0.374        | 0.373        | 0.373        | 0.373        | 0.373        | 0.373        | 0.373        | 0.373        | 0.373        |
| Treatment time, hrs.                   | 4            | 4            | 4            | 4            | 4            | 4            | 4            | 4            | 4            |
| Initial sulfur, wt. percent            | 1.46         | 1.35         | 1.19         | 1.11         | 1.24         | 1.36         | 1.30         | 1.44         | 1.36         |
| Initial ash, wt. percent               | 0.2          | —            | 4.07         | 2.49         | 1.69         | 0.97         | 0.69         | 0.9          | —            |
| Final sulfur, wt. percent              | 0.63         | 0.82         | 0.28         | 0.32         | 0.50         | 0.5          | 0.70         | 0.63         | 0.98         |
| Wt. loss on treatment, percent         | 14           | 3.5          | 6.0          | 6.8          | 4.3          | 5.72         | 4.31         | 1.75         | 5.66         |
| Percent sulfur removed                 | 56.85        | 39.26        | 76.47        | 71.17        | 59.68        | 63.24        | 46.15        | 56.25        | 27.94        |
| Final ash, wt. percent                 | 1.39         | —            | —            | 1.7          | —            | 0.79         | 0.80         | 0.82         | 0.8          |
| Run number                             | 10           | 11           | 12           | 13           | 14           | 15           | 16           | 17           | 18           |
| Particle size                          | -30+100      | -30+100      | -30+100      | -30+100      | -30+100      | -30+100      | -12+30       | -4+12        | -30+100      |
| Percent $\text{Na}_2\text{CO}_3$ added | 0.7          | 0.7          | 0.7          | 0.66         | 0.66         | 0.7          | 0.7          | 0.7          | 0.7          |
| Fluidizing gas                         | $\text{H}_2$ | $\text{H}_2$ | $\text{H}_2$ | $\text{H}_2$ | $\text{H}_2$ | $\text{H}_2$ | $\text{H}_2$ | $\text{H}_2$ | $\text{H}_2$ |
| Temperature, °F                        | 1,200        | 1,400        | 1,600        | 1,200        | 1,200        | 1,200        | 1,200        | 1,200        | 1,200        |
| Pressure, atm                          | 1            | 1            | 1            | 1            | 1            | 1            | 1            | 1            | 1            |
| Velocity of gas, ft./sec.              | 0.373        | 0.373        | 0.373        | 0.373        | 0.746        | 1.12         | .373         | .373         | .373         |
| Treatment time, hrs.                   | 4            | 4            | 4            | 4            | 4            | 4            | 4            | 6            | 8            |
| Initial sulfur, wt. percent            | 1.36         | 1.27         | 1.27         | 1.34         | 1.34         | 1.36         | 1.3          | 1.3          | 1.35         |
| Initial ash, wt. percent               | —            | —            | —            | —            | —            | —            | .71          | .71          | .53          |
| Final sulfur, wt. percent              | 0.58         | 0.67         | 0.97         | 0.55         | 0.54         | 0.61         | 0.58         | .81          | 0.53         |
| Wt. loss on treatment, percent         | 5.66         | 5.0          | 4.34         | 5.7          | 5.23         | 3.2          | 3.7          | 3.43         | 6.0          |
| Percent sulfur removed                 | 57.35        | 47.24        | 23.62        | 58.96        | 59.7         | 55.15        | 55.38        | 37.69        | 57.78        |
| Final ash, wt. percent                 | 0.5          | 0.7          | 0.9          | —            | 0.6          | 0.61         | 0.57         | .54          | .99          |

\*Added to coke.

It can be seen that if the sodium carbonate is added to the coker feedstock (rather than to the coke itself as in Ser. No. 799,151), equivalent results can be obtained using less sodium carbonate, which is important as an ash content of over 1.0 percent is undesirable. As indicated by Run No. 4, a high percentage of sulfur is removed using 5 percent sodium carbonate, but a high ash content is obtained. The ash content can be reduced, as for example by an acid wash, but such a treatment is an added expense. This is why I prefer to use 1 percent or less sodium carbonate (based on coke but added to the coker feedstock).

Table II

#### EFFECT OF TREATMENT WITH HYDROGEN AND NO SODIUM CARBONATE

| Run Number              | 20      | 21      | 22      | 23      |
|-------------------------|---------|---------|---------|---------|
| Particle Size           | -50+100 | -50+100 | -50+100 | -50+100 |
| Temperature, °F         | 1600    | 1400    | 1200    | 1000    |
| Pressure, atm           | 1       | 1       | 1       | 1       |
| Hydrogen, vel.ft/sec    | 0.44    | 0.44    | 0.44    | 0.44    |
| Treatment time, hrs     | 4       | 4       | 4       | 4       |
| Initial sulfur, wt %    | 1.32    | 1.32    | 1.32    | 1.32    |
| Final sulfur, wt %      | 1.08    | 0.94    | 0.79    | 1.29    |
| Initial V.M., wt %      | 8.53    | 8.53    | 8.53    | 8.53    |
| Final V.M., wt %        | —       | 1.61    | 4.16    | —       |
| Loss on treatment, wt % | 10.29   | 11.42   | 8.57    | 5.72    |
| % sulfur removed        | 18.18   | 28.79   | 40.15   | 2.27    |

another crude resid or some other feedstock, the optimum could be at 1,400° or 1,600°F. The invention method would show similar improvement but the optimum would then be 1,400° or 1,600°F, respectively (see Runs 29 and 30).

Treatment of a mixture of sodium carbonate and coker feedstock with an inert gas such as nitrogen (instead of hydrogen), under comparable conditions of temperature and time, does not give the degree of desulfurization which is obtained when sodium carbonate and the hydrogen treatment is used in accordance with my process.

Table III shows the results of desulfurization of high sulfur coke using my process.

55

TABLE III

#### DESULFURIZATION OF HIGH SULFUR COKE

| Run Number                                  | 24          | 25      | 26      | 27      | 28      |
|---------------------------------------------|-------------|---------|---------|---------|---------|
| Particle Size                               | -30+100+100 | -30+100 | -30+100 | -30+100 | -30+100 |
| % $\text{Na}_2\text{CO}_3$ Added, % of coke | —           | —       | —       | —       | —       |
| Temperature, °F                             | 1,200       | 1,200   | 1,200   | 1,200   | 1,200   |
| Velocity, Ft./Sec                           | 0.373       | 0.373   | 0.373   | 0.373   | 0.373   |

|                         | 5    |       |       |       | 6                  |      |      |      |
|-------------------------|------|-------|-------|-------|--------------------|------|------|------|
| Treatment Time, Hrs.    | 4    | 4     | 12    | 16    | Final sulfur, wt % | 0.54 | 0.50 | 0.12 |
| Initial Sulfur, Wt. %   | 4.18 | 4.38  | 4.32  | 4.32  | Wt % loss          | 6.0  | 5.6  | 5.72 |
| Initial Ash, Wt. %      | 0.2  | 0.93  | 0.93  | 0.67  | % sulfur removed   | 57.5 | 61.5 | 75.0 |
| Final Sulfur, Wt. %     | 2.32 | 2.15  | 2.06  | 1.09  |                    |      |      |      |
| Final Ash, Wt. %        | 1.22 | 0.36  | 0.24  | 0.88  |                    |      |      |      |
| Wt. % Loss on Treatment | 2.86 | 2.6   | 5.7   | 8.96  |                    |      |      |      |
| % Sulfur Removed        | 44.5 | 50.91 | 52.31 | 74.77 |                    |      |      |      |
|                         |      |       |       | 76.25 |                    |      |      |      |

The process of this invention has the following advantages over the one described in my co-pending application Ser. No. 799,151 (in which sodium carbonate is added to the coke rather than to the coker feedstock).

1. Sodium carbonate is well distributed in the coke because it can be mixed effectively in the liquid phase. This reduces the amount of sodium carbonate required for the desired sulfur reduction.
2. The ash content of the coke can be maintained at low levels. This is because only a small amount of sodium carbonate is required. The data of Table I show the above two advantages of the process.

The sodium carbonate added to the coker feedstock is distributed in the entire coke. It probably catalyzes the cracking of sulfur compounds in the coke when treated with hydrogen at elevated temperatures. Thus, most of the sulfur comes out as  $H_2S$  during the hydrogen treatment step.

Using a different coke prepared from different coker feedstocks, the following results were obtained using the process of the invention. Runs 29 and 30 were on the same coke prepared from a reduced crude, whereas Run 31 was with a coke prepared from a thermal tar.

TABLE IV

| Run Number           | 29      | 30      | 31      |
|----------------------|---------|---------|---------|
| Particle size        | -50+100 | -50+100 | -50+100 |
| % $Na_2CO_3$ added   | 5.4     | 5.4     | 2.85    |
| Temperature, °F      | 1,200   | 1,600   | 1,200   |
| Velocity, Ft/Sec     | 0.373   | 0.373   | 0.373   |
| Time, Hrs.           | 4       | 4       | 4       |
| Initial sulfur, wt % | 1.27    | 1.30    | 0.48    |

From Runs 29 and 30 it can be seen that with this particular coke, the better hydrogenation temperature was 1,600°F. Run 31 is included to show the operability of the invention using a different type of feedstock.

What is considered new and inventive in the present invention is defined in the hereunto appended claims, it being understood, of course, that equivalents known to those skilled in the art are to be construed as within the scope of the invention. For example, any conventional coker feedstock, as discussed under "Background," may be used. Bicarbonates, sesquicarbonates, or hydrates of carbonates could be used in place of carbonates and are referred to simply as "carbonates."

What is claimed is:

1. A process of producing petroleum coke of reduced sulfur content comprising the steps of adding from about 0.3 to about 5 weight percent of an alkali metal carbonate, based upon coke obtained, to a liquid hydrocarbon coker feedstock, coking the resulting mixture, recovering the coke in a particle size of less than 12 U.S. Standard mesh suitable for fluidizing, and treating in the presence of hydrogen the recovered coke in a fluidized state for at least 2 hours at a temperature of about 1,000°F. to about 2,000°F.

2. The process of claim 1 wherein the coke is subjected to grinding to produce a suitable particle size for hydrogenation.

3. The process of claim 2 wherein the coke is reduced to particle size of less than 12 U.S. Standard mesh.

4. The process of claim 3 wherein the coke is heated at a temperature in the range of about 1,100°F. to about 1,600°F.

5. The process of claim 4 wherein the coke is washed with water after it is treated with hydrogen.

6. The process of claim 5 wherein the alkali metal carbonate is sodium carbonate.

7. The process of claim 6 wherein the temperature of treating with hydrogen is in the range of about 1,100°F. to about 1,400°F.

\* \* \* \* \*